

Feb. 26, 1963

A. W. O. WEBB ET AL

3,079,252

COPPER-BASE ALLOYS

Filed Jan. 9, 1961

2 Sheets-Sheet 1



FIG. I

Inventors  
Alfred W. O. Webb,  
Norman Bailey,  
Roy T. Southin  
by Sommers & Young  
Attorneys

Feb. 26, 1963

A. W. O. WEBB ETAL

3,079,252

COPPER-BASE ALLOYS

Filed Jan. 9, 1961

2 Sheets-Sheet 2



FIG.2

Inventors  
Alfred W.O. Webb,  
Norman Bailey,  
Roy J. Southwick  
by Sommers & Young  
Attorneys

1

3,979,252

## COPPER-BASE ALLOYS

Alfred William Owen Webb, Norman Bailey, and Roy Thomas Southin, Charlton, London, England, assignors to J. Stone & Company (Propellers) Limited, London, England

Filed Jan. 9, 1961, Ser. No. 81,470

Claims priority, application Great Britain Jan. 25, 1960  
13 Claims. (Cl. 75—161)

This invention concerns improvements relating to copper-base alloys containing manganese, aluminium and iron, and also nickel and/or tin.

In the specification of United States Patent No. 2,715,577 we disclosed an alloy containing 10 to 15% of manganese, 6.5 to 9% of aluminium, 2 to 4% of iron and 1.5 to 6% of nickel, and in the specification of United Kingdom Patent No. 809,973, a modification of that alloy in which the aluminium content is less than 6.5%, but not less than 3.5%. These alloys have good casting and welding characteristics, as well as good mechanical properties.

It has now been found that good mechanical properties can be obtained using contents of manganese in excess of 15%, provided that manganese of high purity is employed, and that outstandingly good properties can be obtained within a comparatively narrow range of composition hereinafter referred to.

A copper-base alloy in accordance with the present invention has a basically duplex character, consisting mainly of an alpha phase and a beta phase, and consists essentially of appreciably more than 15% and up to 35% of high-purity manganese, 3.5 to 9.5% of aluminium, 2 to 4% of iron, not more than 6% of nickel and/or not more than 2% of tin, the minimum content of nickel being 1% when no tin is present and the minimum content of tin when no nickel is present being 0.25% while the minimum total of the nickel content plus four times the tin content is not less than 1% when both are present, and the aluminium equivalent (as hereinafter defined) of the aluminium and the manganese present lying within the range 9 to 12%. For most purposes, the manganese content will be not more than 20%, the aluminium content not more than 9% and the aluminium equivalent not more than 11.5%.

Alloys having a very good combination of properties for the production of castings such as marine propellers will have an aluminium equivalent of about 10%.

The effect of variation in manganese content on the structure and properties of the alloy is considerably less than that of variation in aluminium content, but is proportional over the whole range of alloy compositions considered. It is possible therefore to give to manganese an aluminium-equivalent value similar to the zinc-equivalent values recognized by metallurgists practising with high-tensile brasses. We have found that the aluminium-equivalent value of manganese in these copper-manganese-aluminium alloys is 0.16 and this value is to be assumed as the basis for the aluminium equivalents referred to in this specification. The aluminium equivalent of the aluminium and manganese is the sum of the actual percentage of aluminium present plus the aluminium equivalent of the manganese present.

To obtain the most useful mechanical properties for marine-propeller manufacture, it is necessary to maintain a substantially constant alpha/beta ratio in the alloy (about 55%—60% alpha), which can be achieved by reducing the aluminium content as the manganese content is raised.

An alloy of this type containing 15.58% manganese and 7.46% aluminium (aluminium equivalent 9.95%) had a fatigue limit in air of  $\pm 16.5$  tons/sq. in. and a

2

corrosion fatigue limit in sea water, based on 100,000,000 stress reversals, of  $\pm 8.7$  tons/sq. in. This alloy has also been shown to have a very high resistance to corrosion of the impingement type.

For the necessary purity of the alloy, use will be made of high-purity manganese, for example electrolytic manganese, and subsequent contamination will be avoided. Contamination with carbon is particularly to be avoided. Small amounts of carbon in excess of 0.01%, have a marked influence on the tensile properties of the alloy, as is indicated by the following table:

| Aluminium Equivalent, percent | Carbon, percent | 0.15% Proof Stress, tons/sq. in. | Tensile Strength, tons/sq. in. | Elongation, percent |
|-------------------------------|-----------------|----------------------------------|--------------------------------|---------------------|
| 9.52                          | 0.010           | 21.3                             | 45.5                           | 30                  |
| 9.69                          | 0.024           | 20.7                             | 43.2                           | 15                  |

The carbon content should therefore be held to less than 0.02%.

The diagram shown in FIGURE 1 of the accompanying drawings illustrates lower limits of aluminium and manganese contents for alloys with strengths of over 45 and 47.5 tons per sq. in. (curves *a* and *b* respectively) and elongation values over 25 and 20% (curves *c* and *d* respectively).

Alloys with very good properties for marine propellers in particular lie about a line extending from *e* (7.6% aluminium/15% manganese) to *f* (4.4% aluminium/35% manganese). The properties of three typical examples of alloys are as follows:

|                                   | Alloy 1 | Alloy 2 | Alloy 3 |
|-----------------------------------|---------|---------|---------|
| Manganese, percent                | 15.6    | 20.1    | 35.0    |
| Aluminium, percent                | 7.6     | 6.7     | 5.0     |
| Aluminium equivalent, percent     | 10.1    | 9.9     | 10.6    |
| 0.15% Proof Stress (tons/sq. in.) | 23.3    | 23.3    | 22.8    |
| Tensile Strength (tons/sq. in.)   | 49.8    | 47.5    | 43.2    |
| Elongation, percent               | 24      | 25      | 27      |
| Brinell Hardness No. (10/1000)    | 185     | 193     | 166     |

Alloys intended for castings other than marine propellers may require to have different combinations of properties, some requiring to be harder and stronger and others more ductile. Referring to the diagram shown in FIGURE 2 of the accompanying drawings, alloys having the composition limits indicated by the parallelogram *g*, lying on both sides of a line *AB* (indicating alloys with an aluminium equivalent of 10), have properties of considerable use for various purposes in the engineering industry. By way of examples, the properties of two alloys, one of high strength and the other of great ductility are given below:

|                                   | Alloy 4 | Alloy 5 |
|-----------------------------------|---------|---------|
| Manganese, percent                | 19.7    | 15.9    |
| Aluminium, percent                | 7.6     | 6.7     |
| Aluminium equivalent, percent     | 10.8    | 9.3     |
| 0.15% Proof Stress (tons/sq. in.) | 32.8    | 18.8    |
| Tensile Strength (tons/sq. in.)   | 53.7    | 41.8    |
| Elongation, percent               | 12½     | 38      |
| Brinell Hardness No. (10/1000)    | 218     | 150     |

In all the above examples, the iron content is maintained within the range 2—4% and nickel within the range 0—6%.

Although the alloys possess excellent resistance to corrosion and erosion, this can be improved still further by the addition of tin. The extent to which advantage can be taken of this is limited in alloys containing less than 15% manganese because the additions cause loss of ductility. It has been found that larger additions of tin can be accommodated in alloys of higher manganese

content, while still maintaining high ductility, as the following table shows:

| Manganese, percent | Tin, percent | 0.15% Proof Stress, tons/sq. in. | Tensile Strength, tons/sq. in. | Elongation, percent |
|--------------------|--------------|----------------------------------|--------------------------------|---------------------|
| 11.8               | 0            | 18.5                             | 44.4                           | 35                  |
| 11.8               | 0.46         | 18.3                             | 43.5                           | 26                  |
| 11.8               | 0.92         | 18.5                             | 35.8                           | 14                  |
| 15.6               | 0            | 24.4                             | 46.9                           | 28                  |
| 15.6               | 1.04         | 24.6                             | 47.0                           | 26                  |
| 15.6               | 1.56         | 23.9                             | 46.5                           | 25                  |
| 15.6               | 2.08         | 27.1                             | 43.8                           | 13                  |

Additions of up to 2% tin may be made to improve corrosion resistance.

Some alloys of low ductility can be given a low temperature heat treatment to produce combinations of very high proof stress and reasonable ductility. For example, it is possible to obtain an alloy with a 0.15% proof stress of about 40 tons/sq. in. and an elongation of 3%. Wrought alloys of this type can be heat-treated to produce excellent combinations of strength and ductility, the following being typical:

|                              | 0.15% Proof Stress, tons/sq. in. | Tensile Strength, tons/sq. in. | Elongation, percent |
|------------------------------|----------------------------------|--------------------------------|---------------------|
| As forged.....               | 30.4                             | 57.1                           | 11                  |
| Forged and heat-treated..... | 34.8                             | 56.6                           | 16                  |

We claim:

1. A copper-base alloy having a basically duplex character, consisting mainly of an alpha phase and a beta phase and consisting essentially of more than 15% and up to 35% manganese, 3.5 to 9.5% of aluminium, 2 to 4% of iron, and 1 to 6% of nickel, the aluminium-equivalent of the aluminium and the manganese present lying within the range 9 to 12% where the aluminium-equivalent of manganese is 0.16, and having a carbon content as an impurity of less than 0.02%.
2. An alloy according to claim 1, wherein the manganese content is not more than 20%, the aluminium content not more than 9% and the aluminium equivalent not more than 11.5%.
3. An alloy according to claim 1 for the production of castings such as marine propellers, wherein the aluminium equivalent is about 10%.
4. An alloy according to claim 1, wherein the aluminium and manganese contents lie within the limits 7.6% aluminium and 15% manganese on the one hand and 4.4% aluminium and 35% manganese on the other hand.

5. A copper-base alloy having a basically duplex character, consisting mainly of an alpha phase and a beta phase and consisting essentially of more than 15% and up to 35% of manganese, 3.5 to 9.5% of aluminium, 2 to 4% of iron and 0.25% to 2% of tin, the aluminium-equivalent of the aluminium and the manganese present lying within the range 9 to 12% when the manganese-equivalent of aluminium is 0.16, and having a carbon content as an impurity of less than 0.02%.

10 6. An alloy according to claim 5, wherein the manganese content is not more than 20%, the aluminium content not more than 9% and the aluminium equivalent not more than 11.5%.

7. An alloy according to claim 5 for the production 15 of castings such as marine propellers, wherein the aluminium equivalent is about 10%.

8. An alloy according to claim 5, wherein the aluminium and manganese contents lie within the limits 7.6% aluminium and 15% manganese on the one hand and 20 4.4% aluminium and 35% manganese on the other hand.

9. A copper-base alloy having a basically duplex character consisting mainly of an alpha phase and a beta phase and consisting essentially of more than 15% and up to 35% of high-purity manganese, 3.5 to 9.5% of aluminium, 2 to 4% of iron, and at least one element of the group consisting of nickel and tin, the amount of nickel being not more than 6% and the amount of tin being not more than 2%, the minimum total of the nickel content plus four times the tin content being at least 1%, 25 and the aluminium-equivalent of the aluminium and the manganese present lying within the range from 9 to 12% where the aluminium-equivalent of manganese is 0.16, and having a carbon content as an impurity of less than 0.02%.

35 10. An alloy according to claim 9, wherein the manganese content is not more than 20%, the aluminium content not more than 9% and the aluminium equivalent not more than 11.5%.

11. An alloy according to claim 9 for the production 40 of castings such as marine propellers, wherein the aluminium equivalent is about 10%.

12. An alloy according to claim 9, wherein aluminium and manganese contents lie within the limits 7.6% aluminium and 15% manganese on the one hand and 4.4% 45 aluminium and 35% manganese on the other hand.

13. An alloy according to claim 9, wherein the proportion of the alpha phase is about 55-60% of the alloy.

References Cited in the file of this patent

50 UNITED STATES PATENTS

2,715,577 Payne et al. \_\_\_\_\_ Aug. 16, 1955